

# United States Patent Office.

WILLIAM COMPTON, OF NEW YORK, N. Y.

*Letters Patent No. 91,090, dated June 8, 1869.*

## IMPROVED COMPOSITION-CRAYON.

The Schedule referred to in these Letters Patent and making part of the same.

*To all whom it may concern:*

Be it known that I, WILLIAM COMPTON, of the city and State of New York, have invented and made a new and useful Composition for Crayons; and I do hereby declare the following to be a correct description of the said invention, showing the peculiarity of my said composition.

Chalk crayons, employed in schools and academies, are of a very dusty nature, and soil the clothing, the person, and the room, besides being detrimental to health in consequence of breathing the air filled with these fine particles.

The object of this invention is to prevent the dust heretofore arising from crayon-drawing or writing upon a black-board or slate, and at the same time maintain the softness of the crayon, and prevent injury to the black-board or slate.

The composition I make use of has to vary slightly in the proportions, in order that the crayons may be adapted to a wooden surface, a painted surface, or a slate surface, as the slate surface requires a crayon that is harder than those for wood.

The ingredients I employ are Paris-white, or similar white earthy material, starch, and soap; and to harden the crayon and render it adapted to slates, I employ glue or gum.

For a soft crayon I make use of the following ingredients:

About six pounds white.

About three and six-eighths ounces starch.

About three ounces soap.

About one-half ounce gum or glue.

For a harder crayon, adapted to slate surfaces, the proportions should be varied by using about two and one-quarter ounces of glue or gum instead of half an ounce.

The starch and soap are to be dissolved in hot water, sufficient in quantity for rendering the white material plastic for pressing or moulding into shape.

The white should be sifted so as to separate any lumps, and render the plastic mass uniform in its character.

In soft crayons the glue or gum might be dispensed with.

Crayons formed in this manner are used with great facility, because the white dust is prevented from rubbing off on the fingers, and there is little or no dust flying about in the atmosphere when the board or slate is cleaned off, because the particles adhere sufficiently to cause them to fall or to adhere to the rubber.

I find that it is preferable to form the crayons into a cylindrical shape by rolling them upon a table with a flat board, so as to compress and harden the material, and give a slight gloss to the surface, that prevents the chalk rubbing off on the fingers.

The crayons are to be dried either in the sun or by artificial heat.

What I claim, and desire to secure by Letters Patent, is—

The composition for crayons formed of the materials, and as herein set forth.

Also, to the crayon formed by rolling the plastic mass between two surfaces, to consolidate the same, as set forth.

In witness whereof, I have hereunto set my signature, this 15th day of May, A. D. 1869.

WM. COMPTON.

Witnesses:

GEO. D. WALKER,

GEO. T. PINCKNEY.